

# UNITED STATES PATENT OFFICE.

CHARLES F. MCKENNA, OF NEW YORK, N. Y.

## EXPLOSIVE.

1,311,171.

Specification of Letters Patent. Patented July 29, 1919.

No Drawing. Application filed August 22, 1914, Serial No. 858,047. Renewed September 28, 1918. Serial No. 256,145.

*To all whom it may concern:*

Be it known that I, CHARLES F. MCKENNA, a citizen of the United States of America, and a resident of the city of New York, borough of Manhattan, county of New York, and State of New York, have invented certain new and useful Improvements in Explosives, of which the following is a specification.

- 10 The object of the invention is to provide an explosive especially useful in agricultural practice by reason of its strength, its safe conditions, and the simplicity of its manipulation in the open and shallow operations of such applications as distinguished from quarry, mining and tunneling operations where drill holes are deep and hazards of missed shots and other accidents are serious. A further object is to provide an explosive which can be readily manufactured at the site of use and shortly before use, thereby avoiding the necessity for storage or transportation of materials in an explosive condition.
- 15 To this end the materials are preferably initially carried in two containers, one container having in finely pulverized form ammonium perchlorate, and the other container holding in liquid form ingredients which are absorbed by the ammonium perchlorate and form with it the complete explosive. The preferred liquid ingredient is a compound consisting of one part of a mixture of nitrated tar oils obtained from the
- 20 nitration of oils separated from wood tar by fractional distillation and consisting essentially of hydrocarbons and phenols, with two parts of carbon bisulfid, to which is preferably but not necessarily added one
- 25 part of nitrobenzol, and dissolved therein one part of dinitrobenzol. The completed

explosive is preferably formed at the site of use by adding to seventy-five parts of the ammonium perchlorate twenty-five parts of the mixed ingredient in liquid form as above set forth.

In place of nitrobenzol and dinitrobenzol may be substituted their equivalents as reducing agents in nitrated oils of tar obtained as above described, being the distillate coming off after the pyrolytic acid has been distilled off up to the point when a residue of pitch remains.

These nitrated oils are cheaper than any other nitro-body known, being made from wood tar which has so small commercial value that it generally is burned as a fuel. As an ingredient of my explosive these nitrated oils serve the purpose as well as definite nitro-compounds which hitherto have been used. They have also the advantage over nitrated oils from coal tar in that coal tar is more costly than wood tar, and also because such oils from coal tar require elaborate preparation before they are in a condition for use.

What I claim as new, and desire to secure by Letters Patent of the United States, is—

An explosive consisting of seventy-five parts of ammonium perchlorate, five parts of nitrated oils obtained by nitration of oils separated by fractional distillation from wood tar, five parts of nitrobenzol, five parts of dinitrobenzol, and ten parts of carbon bisulfid, substantially as described.

Signed by me at New York, borough of Manhattan, N. Y., this 21st day of August, 1914.

CHARLES F. MCKENNA.

Witnesses:

A. D. GARDIOL,  
CHARLES F. MCKENNA, Jr.